

Aug. 15, 1944.

A. LYEM

2,355,738

ORNAMENTAL MATERIALS

Filed Sept. 3, 1941



INVENTOR

Arthur Lyem

BY

J. Seligman and B. Levinson

ATTORNEYS

## UNITED STATES PATENT OFFICE

2,355,738

## ORNAMENTAL MATERIALS

Arthur Lyem, Cumberland, Md., assignor to  
 Celanese Corporation of America, a corporation  
 of Delaware

Application September 3, 1941, Serial No. 409,341

11 Claims. (Cl. 8—115)

This invention relates to ornamental materials, and more particularly to the production of pattern effects upon a material in web form, such as films and fabrics, having a basis of an organic derivative of cellulose.

An object of my invention is the production of pattern effects upon a material in web form having a basis of an organic derivative of cellulose in an expeditious and economical manner.

Another object of my invention is the production of ornamental materials wherein the pattern or design on said ornamental materials is permanent and highly resistant to laundering and other cleansing operations.

Other objects of my invention will appear from the following detailed description and the accompanying drawing.

Ornamental fabrics presenting a variety of patterned effects have been prepared by weaving said fabrics on special looms such as the Jacquard loom or by making the fabrics on various lace-making machines. As a result, when these patterned fabrics are woven they are quite costly, unless made in large quantities. Because of the fact that the setting-up and operation of looms and machines of this type must be modified for each particular pattern that is woven, and is a highly complicated and costly procedure, the looms and machines are not changed frequently.

I have now discovered that ornamental materials in web form, such as films or fabrics, having a basis of an organic derivative of cellulose may be prepared in a continuous process inexpensively by locally printing said materials with a removable resist compound, subjecting said printed materials to the action of a non-volatile plasticizer for the organic derivative of cellulose dissolved in a suitable volatile solvent for said plasticizer, which solvent has at least some softening action on the organic derivative of cellulose, and then drying said treated material at an elevated temperature. The resist-free portions of the materials are acted upon by the plasticizer and the volatile solvent in which it is dissolved. This treatment produces a pronounced, clearly defined pattern in the materials, the resist-free portion, in the case of a fabric, acquiring an organdie-like finish and the resist-coated portions remaining substantially unchanged. After the materials have been dried they may be washed to remove the resist or, in some cases where the resist is flexible and transparent it may be permitted to remain on the material. The resulting film or fabric presents

5 a highly desirable ornamental patterned effect which, in a fabric which has been treated, is quite similar in appearance to fabric woven on a Jacquard loom or made on lace machines. By printing the film or fabric with the resist compound in any desired pattern an unlimited variety of patterned effects may be obtained, which effects are substantially permanently set in the material and highly resistant to laundering or other cleansing. Since the resist may be applied in a relatively simple manner as by the use of screens, stencils, blocks, rollers, etc., the patterned materials may be produced expeditiously and at comparatively low cost. In lieu of applying the resist to a fabric in a predetermined pattern, it may also be applied at random along the length of the yarns before they are formed into a fabric and the resulting fabric may then be subjected to treatment with plasticizer and to a finishing treatment, yielding a fabric having an unusual overall patterned effect.

10 Various removable resist compounds may be employed in the preparation of the novel films and fabrics of my invention. These resists may be any suitable water-soluble compound, e. g. resins such as those obtained from polyvinyl alcohol, gums such as gum arabic, or protein materials such as albumen and casein.

15 The non-volatile plasticizers which may be employed in treating the resist-printed organic derivative of cellulose materials in accordance with my invention may be, for example, dimethoxyethyl phthalate, dimethyl phthalate, dibutyl tartrate, dibutyl phthalate, ethyl phthalyl ethyl glycolate, triethyl citrate, mono-ethyl-p-toluenesulfonamide, triphenyl phosphate, tricresyl phosphate, diethyl phthalate, methyl phthalyl ethyl glycolate, triacetin and tripropionin. Suitable volatile solvents for the plasticizers which have some softening action on the organic derivative of cellulose of the film or fabric are, for example, ethyl alcohol, methyl ethyl ketone, and acetone.

20 The non-volatile plasticizer and the solvent in which it is dissolved may be used in varying ratios when preparing the solutions which are to be employed for treating the resist printed films and fabrics. The plasticizer may be employed in such amount that it comprises from 5 to 50% by volume of the treating solution. Preferably, however, I employ the plasticizer in amounts ranging from 20 to 40% by volume with the remainder of the solution comprising the volatile solvent.

25 The degree of action of the plasticizing solu-

tion on the resist-printed film or fabric is dependent on both the length of time during which the plasticizing solution is permitted to act on the film or fabric, the temperature of the solution as it is applied and the manner and temperature of the drying step. I have found that very satisfactory results may be obtained when the plasticizing solution is maintained at from 15 to 30° C. and the contact or immersion time of the film or fabric in the plasticizing solution varies from 1 to 30 seconds. The drying of the treated material or the removal of the volatile solvent is preferably carried out by employing a drying chamber through which air heated to an elevated temperature is circulated. The circulating air may be at a temperature of from 60 to 140° C. but is preferably maintained at from 80 to 100° C.

The fabrics treated in accordance with my invention may be woven, knitted, or netted and may be composed entirely of yarns of an organic derivative of cellulose or they may contain, in addition to the organic derivative of cellulose yarns, yarns of other materials which are unaffected by the plasticizing solutions, such as, for example, yarns of cotton, silk, wool or regenerated cellulose. Furthermore, the fabrics may be composed of or contain yarns which are spun from staple fibers having a basis of an organic derivative of cellulose blended with staple fibers of cotton, silk, wool or regenerated cellulose, so that the resulting spun yarns are only in part affected by the plasticizing solution.

In treating the films and fabrics, the solution of plasticizer in the volatile solvent may be applied in many ways. Bath methods may be employed or, if preferred, the solution may be applied by padding or spraying the same on to the material.

While my invention is of particular application with regard to fabrics made of or containing yarns or fibers of cellulose acetate and to films having a basis of cellulose acetate, other organic esters of cellulose as well as ethers of cellulose may be employed. Examples of other cellulose esters are cellulose propionate, cellulose butyrate and mixed esters such as cellulose acetate-propionate and cellulose acetate-butyrate, while examples of cellulose ethers are ethyl cellulose and benzyl cellulose.

In order further to illustrate my invention, reference may be had to the accompanying drawing wherein there is shown, more or less diagrammatically, apparatus for carrying out my novel process.

In accordance with my invention, a roll 1 of a resist-printed fabric 2, which is woven of yarns of an organic derivative of cellulose, is supported on a shaft 3 and the fabric is passed over a guide roller 4 and into a trough 5 containing a solution 6 which comprises a plasticizer and a suitable volatile solvent therefor. The solution in the trough 5 may be heated or cooled to any desired temperature by suitable heating or cooling means (not shown). The fabric 2 is then passed beneath a guide roller 7 set below the surface of the liquid and then over a guide roller 8 from which roller it passes between squeeze rollers 9 and 10 which remove excess liquid from the fabric. The time during which the fabric is subjected to the action of the plasticizing solution may be varied by extending the path of the moving fabric beneath the surface of the liquid, as by employing a plurality of submerged guide

rolls around which the fabric is passed and thus maintained beneath said plasticizing liquid, by lengthening the trough, or where it is desired to subject the materials to only a limited plasticizing treatment the fabric may be passed between the squeeze rollers 9 and 10 directly without being submerged. Since roller 10 is partly beneath the surface of the solution 6 a limited amount of liquid will be applied thereto. The solution 6

10 may be replenished through a pipe 11 set in a hood 12, which hood covers both the trough and squeeze rollers and is positioned so that it precludes excessive evaporation of the volatile solvent. After passing through the squeeze rollers 15 and 10, the plasticized fabric 2 enters a drying chamber 13. In the drying chamber, the moving fabric passes over a guide roller 14 and, after traversing the length of the chamber passes around another guide roller 15 which reverses 20 the direction of the fabric. The drying effect in the chamber is obtained by means of heated air which is forced into the chamber by suitable blowers through entry ports (not shown) placed at suitable points in the chamber. The solvent-laden air leaves the top of the chamber through an opening 16 and may then be led to a suitable solvent recovery system. The dried, plasticized fabric leaves the drying chamber through the base thereof, passes over a guide roll 17 and 30 plastic fabric roll 18 and may then be led to any suitable finishing treatment. While the apparatus has been described in connection with the treatment of the fabric, it will be appreciated that it is equally applicable to the treatment of films.

In order further to illustrate my invention, but without being limited thereto, the following examples are given:

#### 40

#### Example I

A cellulose acetate fabric of a ninon weave is printed in a floral pattern with a resist comprising 5% of a polyvinyl alcohol resin in water. The fabric is then dried and subjected to the plasticizing and solvent action of a solution of 30 parts by volume of dimethoxyethyl phthalate and 70 parts by volume of ethyl alcohol maintained at 20 to 25° C., the time of treatment being about 5 seconds. After the fabric is passed through the squeeze rollers, as described, it is dried in the drying chamber by means of circulating air which has been heated to 90° C. The fabric is then given a finishing treatment. The resulting fabric presents a pleasing floral design comprising unchanged fabric on a background of fabric which now has a crisp, organdie-like finish.

#### 60

#### Example II

A cellulose acetate fabric of a satin weave is printed in a suitable pattern with a reserve paste of 10% gum arabic. This fabric is then subjected to plasticization with a solution of 25 parts by volume of dimethyl phthalate and 65 parts by volume of xylene and 10 parts by volume of acetone at a temperature of 15 to 20° C. for a period of about 10 seconds. After squeezing, the fabric is dried in a drying cabinet at 100° C. by means of circulating air and the procedure carried out in full width in one continuous operation, after which the material is given a finishing treatment if desired. This fabric which is locally plasticized is semi-stiff and does not fray.

*Example III*

A cellulose acetate film is printed in a suitable design with 10% of albumen in water. This film is then subjected to a plasticizing treatment and to the solvent action of a solution containing 40 parts by volume of triethyl citrate and 60 parts by volume methyl ethyl ketone maintained at a temperature of 25 to 30° C. for about 20 seconds. The film is then passed through suitable squeeze rollers and dried in a drying cabinet by means of circulating air maintained at a temperature of 100 to 120° C. This reserve printed and plasticized film is then given a suitable finishing treatment.

The ornamental films and fabrics prepared in accordance with my invention may be extensively employed where decorative effects are desired. Thus, for example, they may be employed for decorative sheets and wrappings, as lamp shades and, when cut to any desired shape, as place mats for table settings.

It is to be understood that the foregoing detailed description is merely given by way of illustration and that many variations may be made therein without departing from the spirit of my invention.

Having described my invention, what I desire to secure by Letters Patent is:

1. Process for the production of materials presenting ornamental effects, which comprises locally applying a water-soluble resist to sheet material having a basis of an organic derivative of cellulose, treating said sheet material with a solution of a non-volatile plasticizer for said organic derivative of cellulose in a volatile solvent for said plasticizer, said volatile solvent having at least some softening action on said organic derivative of cellulose, so as to effect a softening and plasticizing action on the uncoated portion of said material, drying said material at elevated temperature to remove said volatile solvent and then washing the material to remove said water-soluble resist.

2. Process for the production of materials presenting ornamental effects, which comprises locally applying a water-soluble resist to sheet material having a basis of cellulose acetate, treating said sheet material with a solution of a non-volatile plasticizer for said cellulose acetate in a volatile solvent for said plasticizer, said volatile solvent having at least some softening action on said cellulose acetate so as to effect a softening and plasticizing action on the uncoated portion of said material, drying said material at elevated temperature to remove said volatile solvent and then washing the material to remove said water-soluble resist.

3. Process for the production of materials presenting ornamental effects, which comprises locally applying a polyvinyl alcohol resin resist to sheet material having a basis of an organic derivative of cellulose, treating said sheet material with a solution of a non-volatile plasticizer for said organic derivative of cellulose in a volatile solvent for said plasticizer, said volatile solvent having at least some softening action on said organic derivative of cellulose, so as to effect a softening and plasticizing action on the uncoated portion of said material, drying said material at elevated temperature to remove said volatile solvent and then washing the material to remove said polyvinyl alcohol resin resist.

4. Process for the production of materials presenting ornamental effects, which comprises locally applying a polyvinyl alcohol resin resist

to sheet material having a basis of cellulose acetate, treating said sheet material with a solution of a non-volatile plasticizer for said cellulose acetate in a volatile solvent for said plasticizer, said volatile solvent having at least some softening action on said cellulose acetate, so as to effect a softening and plasticizing action on the uncoated portion of said material, drying said material at elevated temperature to remove said volatile solvent and then washing the material to remove said polyvinyl alcohol resin resist.

5. Process for the production of materials presenting ornamental effects, which comprises locally applying a polyvinyl alcohol resin resist to a material in web form having a basis of an organic derivative of cellulose, subjecting said material to the action of a solution of dimethoxyethyl phthalate in ethyl alcohol so as to effect a softening and plasticizing action on the uncoated portion of said material, drying said material at elevated temperature to remove said volatile solvent and then washing the fabric to remove said polyvinyl alcohol resin resist.

6. Process for the production of fabrics presenting ornamental effects, which comprises locally applying a polyvinyl alcohol resin resist to a fabric containing yarns of cellulose acetate, subjecting said fabric to the action of a solution of dimethoxyethyl phthalate in ethyl alcohol so as to effect a softening and plasticizing action on the uncoated portion of said fabric, drying said fabric at elevated temperature to remove said volatile solvent and then washing the fabric to remove said polyvinyl alcohol resin resist.

7. Process for the production of fabrics presenting ornamental effects, which comprises locally applying a polyvinyl alcohol resin resist to a fabric containing yarns of cellulose acetate, subjecting said fabric to the action of a solution of 30 parts by volume of dimethoxyethyl phthalate in 70 parts by volume of ethyl alcohol so as to effect a softening and plasticizing action on the uncoated portion of said fabric, drying said fabric at elevated temperature to remove said ethyl alcohol and then washing the fabric to remove said polyvinyl alcohol resin resist.

8. Process for the production of fabrics presenting ornamental effects, which comprises locally applying a polyvinyl alcohol resin resist to a fabric containing yarns of cellulose acetate, subjecting said fabric to the action of a solution of 30 parts by volume of dimethoxyethyl phthalate in 70 parts by volume of ethyl alcohol maintained at 20 to 25° C. for from 1 to 30 seconds so as to effect a softening and plasticizing action on the uncoated portion of said fabric, drying said fabric at a temperature of from 80 to 100° C. to remove said ethyl alcohol and then washing the fabric to remove said polyvinyl alcohol resin resist.

9. Process for the production of materials presenting ornamental effects, which comprises locally applying a water-soluble resist to a material in web form having a basis of cellulose acetate, subjecting said material to the action of a solution of dimethyl phthalate in xylene and acetone so as to effect a softening and plasticizing action on the uncoated portion of said material, drying said material at elevated temperature to remove said xylene and acetone and then washing the web material to remove said water-soluble resist.

10. Process for the production of materials presenting ornamental effects which comprises locally applying a water-soluble resist to a mate-

rial in web form having a basis of cellulose acetate, subjecting said material to the action of a solution of triethyl citrate in methyl ethyl ketone so as to effect a softening and plasticizing action on the uncoated portion of said material, drying said material at elevated temperature to remove said methyl ethyl ketone and then washing the web material to remove said water-soluble resist.

11. Process for the production of films presenting ornamental effects, which comprises locally 10

5 applying an albumen resist to a film having a basis of cellulose acetate, subjecting said film to the action of a solution of dimethyl phthalate in xylene and acetone so as to effect a softening and plasticizing action on the uncoated portion of said film, drying said film at elevated temperature to remove said xylene and acetone and then washing said film to remove said albumen resist.

ARTHUR LYEM.